# EUROPEAN PATENT SPECIFICATION

(11) **EP 0 078 701 B1**
(45) Date of publication and mention of the grant of the patent: **15.01.1986**
(21) Application number: 82305812.8
(22) Date of filing: 02.11.1982
(51) Int. Cl.: C10C 3/04

(54) **Process for preparing modified asphalts**
Verfahren zur Herstellung von modifizierten Asphalten
Procédé pour la préparation d'asphaltes modifiés

(30) Priority: 06.11.1981 GB 8133560
(43) Date of publication of application: 11.05.1983
(73) Proprietor: EXXON RESEARCH AND ENGINEERING COMPANY, Florham Park, New Jersey 07932-0390 (US)
(72) Inventor: Chavet, Bernard, F-76150 Notre Dame De Bondeville (FR)
(74) Representative: Pitkin, Robert Wilfred

## Description

This invention relates to a process for preparing a sulfur-modified asphalt. The term asphalt is employed herein synonymously with the term bitumen.

It is known that the addition of sulfur to asphalt leads to modified binders having improved workability and mechanical characteristics. However, the blending operation, which must take place above 120°C (melting point of sulfur), is generally accompanied by the evolution of significant amounts of H₂S. This is due to the reaction of sulfur with some molecules of the asphalt blend which are especially prone to it.

It is an object of the present invention to provide an improved process, giving rise to decreased, or no, H₂S evolution.

According to the present invention there is provided a process for preparing a sulfur-modified asphalt, characterised in that:
(a) the asphalt is contacted with a liquid or gaseous oxidant, optionally in the presence of a catalyst, at a temperature of 140°C to 170°C for a period up to one hour, such that the softening point of the asphalt is not materially altered; and
(b) the resultant product is subsequently contacted with non-chemically-combined or bound sulfur, at a temperature in the range 120°C to 170°C.

It has been found that for the oxidation step (a) of the process of the invention solid oxidants, for example, chromium trioxide and phosphorus. pentasulfide are not suitable. A suitable liquid oxidant is hydrogen peroxide. Preferably, however, the oxidant is air or oxygen.

The normally preferred temperature of contact in step (a) is in the range 145°C to 155°C. The duration of the contact is not more than one hour, typically 10 to 20 minutes depending on the feedstock being processed. The product of step (a) is one in which the softening point of the starting material is not significantly altered.

Thus, the product of this step of the process is a deliberately mildly oxidized asphalt and hence is very different from the well-known oxidized or "blown" asphalt products which are normally prepared by oxidation for from 4 to 8 hours at 240°C to 290°C. The product is also very different from that disclosed in United Kingdom Patent 278,679 published in 1928. The disclosure there is of a tar, tar oil or anthracene oil oxidized with air, or a liquid oxidant such as nitric acid, to an extent that the product (i) retains a sufficient degree of fluidity (ii) is insensitive to water, so that it can be directly used in road construction.

FR 1.567.671-A, broadly discloses a process in which a paraffinic petroleum bitumen is treated at 110 to 150°C, for an unspecified period of time, with air in the presence of certain types of catalysts. There is no reference to, or evidence of, the products so made having reduced reactivity toward sulfur. Moreover, in the only two specific examples relating to the air treatment a temperature of 130°C is employed, either for 1 hour or 2 hours. This is a lower temperature and, in the second case, a longer time than required for step (a) of the process of the present invention.

According to step (b) of the process of the invention, the mildly oxidized product of step (a) is blended with sulfur at a temperature in the range 120°C to 170°C. The steps (a) and (b) are preferably conducted at substantially the same temperature in the range 140°C to 170°C, more especially 145°C to 155°C. The step of contacting with sulfur need not necessarily immediately follow step (a) but can, if desired, follow later, for example, at a road-making site.

The sulfur may be employed in amount from up to 45 wt%, more especially 30 wt%.

The asphalt feedstock employed in processes of the invention may be any one of the known non-oxidized materials, for example, the penetration grade asphalts such as 40/60 to 180/220, preferably 80/100. However, such softer petroleum residua can be employed, for example, those with penetrations of about 600, or higher, including the light 600-800 grade (ASTM D 5).

The invention will now be illustrated by reference to the following Examples:-

### Example 1

In this example ten different asphalt types were tested with respect to their reactivity with sulfur. The reactivity was quantified by the cumulative quantity of H₂S evolved during the first ten minutes of treatment of the asphalt with elemental sulfur at 150°C.

Table 1 shows for each material its crude oil origin, its penetration and the said H₂S quantity evolved.

The first six materials show essentially the same reactivity to sulfur independent of the crude oil origin. Moreover, as indicated by Tests 2 and 3, the reactivity is substantially independent of the penetration, so that short and long run vacuum residua produced from the same crude oil behave substantially similarly when treated with the sulfur.

Tests Nos 7 and 8 were conducted with two different blends of straight run vacuum residua and oxidized vacuum residua, that is to say the normal fully oxidized material. The blends show less reactivity with sulfur under the stated conditions.

Finally, Tests 9 and 10 were conducted with two mildly blown materials made in accordance with step (a) of the invention. Both materials show a considerably reduced reactivity with sulfur under the stated conditions, the origin of crude oil being unimportant. It will be seen that the reactivity is appreciably less than even the blends 7 and 8; indicating that the results obtainable by means of the invention cannot be achieved by mereblend- ing of known blown and un-blown materials.

### Example 2

In order to illustrate suitable conditions for conducting the mild oxidation, a series of air blowing experiments was conducted on some asphalt materials at 150°C or 165°C and for oxidation times in the range 5 to 60 minutes. The asphalts employed were (1) a straight run vacuum residuum from an Arabian Light crude (2) a blend of straight run vacuum residuum having a penetration 80 to 100 and (3) a straight run vacuum residuum of penetration 80 to 100 from an Arabian Heavy crude oil.

Fig. 1 is a plot of relative reactivity of the various oxidized materials thus produced with sulfur, against oxidation time. With all materials H₂S is reduced by 50% after only 15 mins air blowing, and by 75% after 1 hour.

Similar results were obtained employing hydrogen peroxide as the oxidant. By contrast NH₄N0₃, Cr0₃ and P₂0₅ do not produce similar results.

### Example 3

This example illustrates that the mildly oxidized product of step (a) of the invention retains its low reactivity to sulfur over a storage period at 150°C of ten or more days. This is very important in practice in that the oxidized product can be made and hot-stored in one location and thereafter blended with sulfur at another location days later.

Fig. 2 shows the results obtained with an asphalt of penetration 80 to 100 from an Arabian Heavy crude and a residue from the vacuum distillation of an Arabian Light crude. The figure clearly shows that even after 10 days storage, both products are still considerably less reactive with sulfur than the corresponding unblown materials.

The sulfur-modified asphalts of the invention have considerable importance as binding agents in road-making and road-surfacing operations, among other uses. H₂S evolution has hitherto presented problems which sometimes rule out the possibility of using sulfur-modified asphalts even though they have desirable properties. By means of the invention H₂S evolution can be reduced, thereby widening the practical scope of use of sulfur-modified asphalts, since the important properties of those are not significantly affected in the products made according to the present invention.

## Claims

1. A process for preparing a sulfur-modified asphalt, characterised in that:
(a) the asphalt is contacted with a liquid or gaseous oxidant, optionally in the presence of a catalyst, at a temperature of 140°C to 170°C for a period up to one hour, such that the softening point of the asphalt is not materially altered; and
(b) the resultant product is subsequently contacted with non-chemically-combined or bound sulfur, at a temperature in the range 120°C to 170°C.

.2. A process as claimed in claim 1, wherein the oxidant employed in step (a) is oxygen or air.

3. A process as claimed in claim 1 or claim 2, wherein the contacting with the sulfur follows substantially immediately after the contacting with the oxidant.

4. A process as claimed in any preceding claim, wherein the steps (a) and (b) are both conducted at substantially the same temperature, which temperature is in the range 140°C to 170°C, preferably 145°C to 155°C.

5. A sulfur-modified asphalt whenever produced by the process claimed in any preceding claim.

## Patentansprüche

1. Verfahren zur Herstellung eines Schwefelmodifizierten Asphalts, dadurch gekennzeichnet, daß
a) der Asphalt mit einem flüssigen oder gasförmigen Oxidationsmittel, gegebenenfalls in Gegenwart eines Katalysators, bei einer Temperatur von 140 bis 170°C über einen Zeitraum von bis zu einer Stunde so kontaktiert wird, daß sich der Erweichungspunkt des Asphalts nicht wesentlich ändert, und
b) das resultierende Produkt anschließend mit nicht chemisch kombiniertem oder gebundenem Schwefel bei einer Temperatur im Bereich von 120 bis 170°C kontaktiert wird.

2. Verfahren nach Anspruch 1, dadurch gekennzeichnet, daß das in Stufe (a) verwendete Oxidationsmittel Sauerstoff oder Luft ist.

3. Verfahren nach Anspruch 1 oder 2, dadurch gekennzeichnet,, daß sich das Kontaktieren mit dem Schwefel im wesentlichen unmittelbar an das Kontaktieren mit dem Oxidationsmittel anschließt.

4. Verfahren nach einem der vorangehenden Ansprüche, dadurch gekennzeichnet, daß die Stufen (a) und (b) beide bei im wesentlichen derselben Temperatur durchgeführt werden, wobei diese Temperatur im Bereich von 140 bis 170°C und vorzugsweise 145 bis 155°C liegt.

5. Schwefel-modifizierter Asphalt hergestellt nach dem Verfahren gemäß einem der vorangehenden Ansprüche.

## Revendications

1. Procédé de préparation d'un asphalte modifié au soufre, caractérisé en ce que:
(a) l'asphalte est mis en contact avec un oxydant liquide ou gazeux, éventuellement en présence d'un catalyseur, à une température comprise de 140°C à 170°C pendant une durée allant jusqu'à une heure, de sorte que le point de ramollisement de l'asphalte n'est pas sensiblement modifié; et
(b) le produit obtenu est ensuite mis en contact avec du soufre non combiné chimiquement ou non lié, à une température dans le domaine de 120°C à 170°C.

2. Procédé selon la revendication 1, caractérisé en ce que l'oxydant employé dans l'étape (a) est l'oxygène ou l'air.

3. Procédé selon la revendication 1 ou la revendication 2, caractérisé en ce que la mise en contact avec le soufre succède pratiquement immédiatement à la mise en contact avec l'oxydant.

4. Procédé selon l'une quelconque des revendications précédentes, caractérisé en ce que les étapes (a) et (b) sont toutes les deux réalisées pratiquement à la même température, cette température étant comprise dans le domaine de 140°C à 170°C, de préférence de 145°C à 155°C.

5. Asphalte modifié au soufre lorsqu'il est produit par le procédé revendiqué dans l'une quelconque des revendications précédentes.
